

# United States Patent Office

3,535,247

1

3.535.247

5,552,247

**FIBER REACTIVE AND FIBER NON-REACTIVE  
FLUORO-ALKYLACETALS OF DIALDEHYDES  
AND MATERIALS TREATED THEREWITH**

AND MATERIALS TREATED THEREWITH  
Domenick Donald Gagliardi, 185 Howland Road,

Donald Gagliardi, 185 Howland Street, Greenwich, R.I. 02818

East Greenwich, R.I. 02818  
Aug. Continuation of application Ser. No.

583,429, Sept. 30, 1966, which is a continuation-in-part of application Ser. No. 295,507, July 16, 1963.

This application July 7, 1969, Ser. No. 845,641

W.L.G. - GM - 2.10 - 1

## 8 Claims

#### ABSTRACT OF THE DISCLOSURE

Perfluoro diacetals of dialdehydes are provided which are useful for treating substrates in order to obtain oil and water repellent finishes thereon. Of the four ether groups present in the molecule at least one contains a C<sub>3</sub> to C<sub>22</sub> alkyl having a terminal CHF<sub>2</sub> or CF<sub>3</sub> grouping and wherein at least 70% of the normally present hydrogen atoms of the alkyl have been replaced by fluorine atoms. The remaining ether groups may be either similar or different perfluoro alkyl moieties of 3 to 22 carbon atoms or alkyl of 1 to 30 carbon atoms. Where two of the ether groupings on the same carbon atom are alkyl of 1 to 4 carbon atoms, the compounds are reactive with substrates containing active hydrogen therein, e.g. cellulose. The diacetals of this invention are either liquids or high-melting waxes depending upon the molecular weight of the product.

This application is a continuation of application S.N. 583,429, filed Sept. 30, 1966 and now abandoned which is in turn a continuation-in-part of application S.N. 295,507, filed July 16, 1963.

The present invention relates to the preparation of fiber reactive and non-reactive fluoroalkylacetals of di-aldehydes and to textile materials and other substrates to which said fluoroalkylacetals are affixed.

which said hydroalkylacetals are annexed.

The treatment of textile materials to endow the textile with an ability to shed water or repel water dates from at least the early nineteenth century when Macintosh presented to the world his treated cloth having a sufficient water-repellency that his name was used to designate a group of garments known as Macintoshes. From the time of Macintosh to 1935 to 1940 textile materials were coated with various compositions such as rubber, linseed oil-rubber mixtures, synthetic dopes, and other whimsically strange compositions which formed a continuous coating on the woven material and prevented the penetration of water.

Without understanding the basic principles of surface free energy, contact angle and spreading coefficient several unrelated practical developments emerged during the years 1935 to 1940 which changed the art of textile waterproofing. In Germany, especially at Chemische Fabrik Pfereze, a series of paraffin wax emulsions was developed which, when padded onto textiles, produced a high contact angle of water drops on the treated surface and a high degree of shower resistance without changing the porosity or air-permeability of the textile material. The treated fabrics were not wetted by water or water-borne liquids and stains because of the change in free energy of the surfaces of the fiber and not because of closing or plugging the interstices of the fabric. 65

By use of the new wax emulsion-metallic salts compositions, it was then possible to produce fabrics which were water repellent and had the feel and appearance of conventional textiles but did not look like oil-cloths

2

or rubberized coated fabrics. The only practical limitation of such compositions was the durability to washing and dry cleaning. Such wax emulsion-metallic salts compositions usually contain (1) paraffin wax or mixtures of vegetable wax esters such as carnauba, candelilla, or sugar cane wax; (2) an emulsifying agent, generally glue, gelatin and rosin soaps; and (3) an aluminum or zirconium salt usually the formate or acetate. The primary function of the salts is to insolubilize the glue and other emulsifiers after the emulsion is deposited on the fibers.

A large variety of such products are still used as low-cost, non-durable water repellents for textiles. Other than water repellency for rainwear fabrics, such compositions produce fabrics which have a fair degree of spot- and stain-repellency against water-borne stains.

The search for durable or permanent water repellents, especially for cellulosic fibers, was initiated by the deficiencies of the previously discussed wax emulsion-metallic salt products.

20 The first important development was the use of octodecyloxymethyl pyridinium chloride available in England under the trade name "Velan." "Velan" is a quaternary ammonium compound made by the chloromethylation of octadecanol followed by quaternization with pyridine 25 to yield a composition corresponding to the formula:



This structure, unlike other quaternaries, is unstable and under acid conditions reacts with surfaces containing active hydrogen, e.g., the hydrogen of the hydroxyl group of cellulose fibers. This, if Z is the base of the cellulose molecule then the reaction may be represented by the equation



Fabrics treated with such a compound are durably water repellent, are porous, soft, and appear like untreated fabrics. A major improvement in this product was made by du Pont and Warwick Chemical Company, who produced the stearamidomethyl analog of "Velan" having a composition corresponding to the formula



known commercially as "Zelan" and "Norane R." The advantages of the stearamide product is its greater initial water repellency and greater durability to washing. Such products are still in the forefront of the leaders in rainwear fabrics finishes.

The search for fiber reactive or durable water-repellent textile finishes continues. Other classes of water-repellent textile finishes have been introduced to the textile finishing art of which silicone water-repellents methylolstearamide compositions ("Permel," "Ahcovel NW"), hydrophobic resins ("Norane GG," "Ranedare R," "Argus DWR"), octadecylketene dimer ("Aquapel") and others are representative.

While durable water repellents, such as those briefly mentioned hereinbefore, had been initially designed for outerwear and raincoat type applications, in the period

from 1950 to 1956 the use of such products as finishes for men's suitings, dress goods, and upholstery materials became almost common place. In these uses, promotional emphasis was placed not upon water-repellency but upon resistance to spotting and staining. It was subsequently observed that fabrics treated with such water-repellents had a high degree of resistance to soiling by water-borne soils and stains and were easier to launder. The only limitation of such finishes was that they appeared to attract oily soils and the fabrics treated with these finishes were not stain repellent against oily materials such as oils, greases, gravy, mayonnaise, and the like.

While resistance to soiling by water-borne soils and stains, e.g., coffee is of considerable importance, the development of finishes which resist staining by oil-borne stains such as mayonnaise and, particularly finishes which do not attract oily "particulate-soil" open-up an entirely new field of textile finishing. For example, the cocktail party and the canapes served therewith does not concomitantly include the need to dry clean the rugs. Of even greater importance, is the ability of a finish to shed rather than attract oily "particulate-soil." The incidence of staining a shirt-front with mayonnaise is only once or twice a day but the dust, i.e., "particulate-soil" of the environment and the oily exudations of the human skin which deposit on the neckband and wrist-end of the cuffs of men's shirts is always present during each minute of the hours during which the shirt is worn. Thus, it is manifest that, while the disadvantage of these durable water-repellents when used as finishes for men's suitings, dress goods, upholstery and the like may not seem too important upon cursory consideration, after more profound review the boon of finishes which repel not only oil-borne stains but in addition repel rather than attract oily "particulate-soil" becomes self-evident. Such "particulate-soil" repellent finishes are provided by the present novel perfluoroalkylacetals of dialdehydes of the present invention.

The novel perfluoroalkylacetals of dialdehydes of the present invention provide finishes for textile materials of two relatively durable classes, i.e., one class of the present perfluoroalkyl acetals is non-reactive with the fiber, the other class of the present perfluoroalkylacetals is reactive with active hydrogen contained in the surface of the fiber.

#### NON-REACTIVE PERFLUOROACETALS

The perfluoroalkylacetals of the present invention which are non-reactive with the fiber have compositions corresponding to the formula



Where  $Q_1$  is the residue of an alcohol having 3 to 22 carbon atoms, having either a terminal  $-CHF_2$  group or, preferably, a terminal  $-CF_3$  group in which at least 70 percent of the hydrogen atoms of the alkyl group of the parent alcohol are replaced with fluorine atoms and the alkyl chain is straight or branched and  $n$  is zero to 22, and the other  $Q$ 's are similar to  $Q_1$  or an aliphatic chain containing at least 6 uninterrupted carbon atoms, and preferably alkyl of 6 to 30 carbon atoms.

#### REACTIVE PERFLUOROACETALS

The perfluoroacetals of the present invention which are reactive with active hydrogen contained in the surface of the fiber have compositions corresponding to the formula



where  $Q_1$  and  $n$  have the significance given hereinbefore,  $X$  and  $Y$  together may represent  $=O$  (i.e., an aldehyde) or may be independently  $-OR_1$  wherein  $R_1$  is alkyl of 1 to 4 carbons, and  $Z$  may be  $OQ_1$ ,  $-OR_1$  or  $CR_2$  where

$R_2$  is an aliphatic chain containing at least 5 uninterrupted carbon atoms. These fiber-reactive-perfluoroacetals react with the active hydrogen contained in the surface in a manner corresponding to that indicated by the following equation in which  $Z(OH)_m$  represents cellulose having  $m$  active hydrogen atoms in the surface

(a)



(b)



The perfluoroalkylacetals of dialdehydes of the present invention are either liquids or high melting waxes depending on the value of  $(n)$  and on the chain length of the fluoroalcohol ( $Q_1OH$ ).

The preparation of dialdehyde diacetals is described in U.S. Pat. No. 2,556,312. The patentee discloses that the initial overall reaction between an orthoformic ester and open chain alkenyl alkyl ether is a diacetal of malondialdehyde having a structure illustrated by the following formula



where  $R'$  represents an alkyl, cycloalkyl, aralkyl, aryl, halogen-substituted alkyl, alkoxyalkyl, aryloxyalkyl or alkenyl group;  $R^2$  and  $R^3$  represent hydrogen or an alkyl group;  $R^4$  represents an alkyl, cycloalkyl, alkoxyalkyl or halogen-substituted alkyl group or  $R^2$  and  $R^4$  represent a closed hydrocarbon chain  $-(CH_2)_y-$  wherein  $y$  is 2 or 3; and  $R^5$  designates a radical of classes represented by  $R'$  and  $R^4$ .

Such acetals are suitable for producing the compounds of this invention by transesterification with a fluoroalcohol ( $Q_1OH$ ) as hereinafter described. The preferred acetals for use in this reaction are those of the formula:



wherein at least one of the  $R$ 's is lower alkyl, e.g., methyl, ethyl, isopropyl, n-propyl, isobutyl, n-butyl and the others independently among alkyl, e.g.,  $C_1$  to  $C_{30}$  and  $R^2$  and  $R^3$  are as indicated above in Formula III.

Specific acetals as illustrative only of Formula IV include:

- 1,1,2,2-tetraethoxyethane
- 1,1,3,3-tetraethoxypropane
- 1,1,4,4-tetraethoxybutane
- 1,1,5,5-tetraethoxypentane
- 1,1,2,2-tetraisopropoxyethane
- 1,1,6,6-tetraisopropoxyhexane
- 1,1,10,10-tetraisopropoxydecane
- 1,1,12,12-tetraisopropoxydodecane
- 1,1,16,16-tetraisopropoxyhexadecane
- 1,1,20,20-tetraisopropoxyeicosane
- 1,1,20,20-tetraethoxyeicosane
- 1,1-diethoxy-2,2-diisopropoxyethane
- 1,1-diethoxy-2,2-di-decyloxyethane
- 1,1-diethoxy-2,2-di-dodecyloxybutane
- 1,1-diethoxy-2,2-di-n-butoxydecane
- 1,1,2-triethoxy-2-decyloxyethane
- 1-ethoxy-1,2,2-tri-dodecyloxyethane
- 1,1-tetraethoxy-4,4-di-n-octyloxybutane
- 1,1-tetraethoxy-3,3-di(hexyloxyhexyloxy)pentane

The following fluoroalcohols are illustrative of those  $Q_1OH$  compounds which are contemplated herein:

- 1H,1H-pentafluoro-1-propanol
- 1H,1H-heptofluoro-1-butanol
- 1H,1H-nonafluoro-1-pentanol
- 1H,1H-perfluoroisobutanol  $[(CF_3)_2CFCH_2OH]$
- 1H,1H-undecafluoro-1-hexanol
- 1H,1H-tridecafluoro-1-heptanol
- 1H,1H-pentadecafluoro-1-octanol
- 1H,1H-heptadecafluoro-1-nonanol
- 1H,1H-nonafluoro-1-decanol
- 1H,1H-perfluoro-1-dodecanol  $(n-C_{11}F_{23}-CH_2OH)$
- 1H,1H-perfluoro-1-eicosanol  $(n-C_{19}H_{39}CH_2OH)$
- 1H,1H,4H-perfluoro-1-butanol  $H(CF_2)_3CH_2OH$
- 1H,1H,5H-perfluoro-1-pentanol
- 1H,1H,7H-perfluoro-1-heptanol
- 1H,1H,11H-perfluoro-1-undecanol
- 1H,1H,21H-perfluoro-1-henicosanol
- 1H,1H,3H-perfluoro-1-pentanol
- 1H,1H,3H-perfluoro-1-octanol

The preparation of tetra-acetals of glyoxal is described in U.S. Pat. No. 2,360,957. This patentee states that glyoxal tetra-acetals are prepared in economic yields by direct reaction at elevated temperatures of glyoxal with a lower, chloroalkanol to produce the tetra-acetals having a composition represented by the formula



In U.S. Pat. No. 2,681,370 the preparation of perfluoroalkylaldehydealkylhemiacetals having the generic formula



are said to provide a commercially valuable way of transporting the corresponding fluorocarbon aldehyde compounds in pure form. These fluorocarbon aldehydes are described in U.S. Pat. No. 2,568,500. The aforementioned perfluoroalkylaldehydealkylhemiacetals are said to be extremely reactive, readily polymerize and are very sensitive to moisture, forming the corresponding monohydrates (aldehydrols) almost instantaneously in the presence of water.

In U.S. Pat. No. 2,842,601 the preparation of fluorinated hemiacetals is described. This patentee describes the preparation of these hemiacetals, having the generic formula



in which each  $n$  is an integer from 1 to 12, by direct photochlorination of alcohols having the general formula  $\text{H}(\text{CF}_2\text{CF}_2)_n\text{CHOH}$ , in which  $n$  has the same meaning as before, at temperatures of from 0° C. to 80° C. using from 0.1 to 0.5 mol of chlorine per mol of alcohol.

The dialdehyde diacetals described in U.S. Pat. No. 2,556,312 are said to be useful as pharmaceutical intermediates. The tetra-acetals of glyoxal described in U.S. Pat. No. 2,360,957 are said to possess merit as an addition agent for extreme pressure lubricants, in making rubber-like products by condensation with polysulfide compounds, and its plurality of chlorine atoms makes it a valuable intermediate for the synthesis of many compounds of unusual structure and properties.

The only use suggested for the perfluoroalkylaldehyde alkylhemiacetals in U.S. Pat. No. 2,681,370 is a commercially valuable way of transporting the corresponding fluorocarbon aldehyde compounds in pure form.

The fluorinated hemiacetals described in U.S. Pat. No.

2,842,601 are said to be readily converted to the corresponding aldehydes and this makes them valuable as a convenient storage source of aldehydes.

It is also stated that, by chlorination, the omega-chloro-omega'-hydroperfluoro aliphatic hydrocarbons are produced which are known to be useful as intermediates in the preparation of surface active agents and treating agents for paper, textiles, and the like and highly fluorinated compounds useful as heat transfer media and the like as described in U.S. Pats. Nos. 2,790,815 and 2,551,573.

It will be observed that none of the disclosures of the U.S. patents discussed briefly hereinbefore have any discussion of endowing textile materials with the capability to repel rather than attract "particulate-soil."

Yet, as emphasized hereinbefore, probably the most important characteristic of a finish for textile materials such as dress goods, men's suitings, floor coverings, upholstery, and the like is the capability to repel rather than attract "particulate-soil."

20 The perfluoroalkylacetals of dialdehydes can be applied from aqueous emulsions thereof or from solutions thereof in organic solvent. The fabric to which the acetal is to be affixed is contacted with the aqueous emulsion or the solution of the acetal to at least eighty to ninety percent wet pick-up of a solution containing at least one percent solids. Generally below about 0.8% by weight perfluoro compound based on the weight of the fabric does not give optimum results although as little as 0.1% is effective. Up to 10% by weight may be used but preferably not more than about 5% gives maximum benefits. The treated fabric is then cured at a temperature in the range of from room temperature to about 375° F. for a period of time, e.g., five to ten minutes at 300° F.

The perfluoroalkanols, having a terminal  $-CF_2H$  or 35 a terminal  $-CF_3$  group can be reacted with other polyaldehydes such as polyaldehyde starch, condensed acrolein aldehyde. The novel perfluoroalkylketals can be prepared by transesterification of methyl, ethyl, or propyl ketals of the polyaldehydes of starch, condensed acrolein and 40 the like or by direct reaction of the perfluoroalkanol and the polyaldehyde.

#### EXAMPLE 1

Illustrative of the capability of the fluoroalkylacetals 45 of dialdehydes to endow textile materials to which the fluoroalkylacetals are affixed with capability to shed particulate soil and to repel water- and oil-borne stains are the data presented in Table I.

Exemplary of the perfluoroalkylacetals of dialdehydes 50 is that prepared from trihydroxonafluoroalcohol



see U.S. Pat. 2,917,409, Example 1] and malonaldehyde-tetraethylacetal in the mol ratio of two mols of the alcohol to one mol of the acetal.

TABLE I

| 60                    | Treatment of<br>80 x 80 cotton with | Oil<br>repellency | Soil repellency,<br>percent reflectance |    |
|-----------------------|-------------------------------------|-------------------|-----------------------------------------|----|
|                       |                                     |                   | A                                       | B  |
| None (control) -----  |                                     | 0                 | 25                                      | 75 |
| 3% fluoroacetal ----- |                                     | 70                | 38                                      | 78 |

B.—Before washing as described hereinafter.

A.—After washing as described hereinafter.

#### EXAMPLE 2

Example 1 is repeated using the following acetals in dimethylformamide at the indicated concentrations and drying at room temperature.

70 Conc. Reference to Formula I  
A. 1%  $Q_1$  and  $Q_2=H(CF_2)_6CH_2-$ ;  $Q_3$  and  $Q_4=$   
lauryl and  $n=0$   
B. 1%  $Q_1$  and  $Q_2=H(CF_2)_5CH_2-$ ;  $Q_3$  and  $Q_4=$   
isoctyl and  $n=1$

- C. 1%  $Q_1$  and  $Q_2=H(CF_2)_8CH_2-$ ;  $Q_3$  and  $Q_4=$  stearyl and  $n=2$   
 D. 1%  $Q_1, Q_2, Q_3$  and  $Q_4=H(CF_2)_8CH_2-$  and  $n=2$   
 E. 1%  $Q_1$  and  $Q_2=F(CF_2)_4CH_2-$ ;  $Q_3$  and  $Q_4=$  decyl and  $n=3$   
 F. 2%  $Q_1, Q_2, Q_3$  and  $Q_4=F(CF_2)_3CHFCF_2CH_2-$  and  $n=0$   
 G. 4%  $Q_1, Q_2, Q_3$  and  $Q_4=F(CF_2)_3CHFCF_2CH_2-$  and  $n=2$   
 H. 5%  $Q_1, Q_2, Q_3$  and  $Q_4=H(CF_2)_7CH_2-$  and  $n=12$   
 I. 3%  $Q_1$  and  $Q_2=F(CF_2)_6CH_2-$ ;  $Q_3$  and  $Q_4=n$ -hexyl and  $n=18$   
 J. 1%  $Q_1$  and  $Q_2=F(CF_2)_{18}CH_2-$ ;  $Q_3$  and  $Q_4=n$ -heptyl and  $n=0$   
 K. 1%  $Q_1=F(CF_2)_{10}CH_2-$ ;  $Q_2, Q_3$  and  $Q_4=$  lauryl and  $n=0$   
 L. 1%  $Q_1=F(CF_2)_8CH_2-$ ;  $Q_2, Q_3$  and  $Q_4=$  decyl and  $n=4$   
 M. 1%  $Q_1, Q_2$  and  $Q_3=F(CF_2)_7CH_2-$ ;  $Q_4=$  iso-octyl and  $n=0$   
 N. 1%  $Q_1, Q_2$  and  $Q_3=F(CF_2)_7CH_2-$ ;  $Q_4=$  tridecyl and  $n=1$

In all instances excellent oil repellency and soil resistance comparable to Example 1 are obtained. The treated textiles also are characterized by good water-repellent properties.

#### EXAMPLE 3

Example 2 is repeated except that the treated textiles are cured for 5 minutes at 300° F. Similar results are obtained.

#### EXAMPLE 4

Example 2 is repeated using the following compounds:

- Conc. Reference to Formula II  
 A. 1%  $Q_1$  and  $Z=F(CF_2)_8CH_2-$ ; X and Y together are ( $=O$ ) and  $n=0$   
 B. 1%  $Q_1$  and  $Z=F(CF_2)_6CH_2-$ ; X and Y together are ( $=O$ ) and  $n=1$   
 C. 1%  $Q$  and  $Z=F(CF_2)_8CH_2-$ ; X and Y=ethyl and  $n=0$   
 D. 1%  $Q$  and  $Z=F(CF_2)_6CH_2-$ ; X and Y=iso-propyl and  $n=1$   
 E. 3%  $Q$  and  $Z=F(CF_2)_5CH_2-$ ; X=ethyl; Y=lauryl and  $n=0$   
 F. 3%  $Q=H(CF_2)_8CH_2-$ ; Z=decyl; X and Y=ethyl and  $n=0$   
 G. 4%  $Q=H(CF_2)_8CH_2-$ ; Z=octyl; X and Y together are ( $=O$ ) and  $n=0$   
 H. 5%  $Q$  and  $Z=F(CF_2)_4(CHF)_2CH_2CH_2-$ ; X and Y=ethyl and  $n=0$   
 I. 2%  $Q$  and  $Z=H(CF_2)_5(CHF)_3CF_2CH_2-$ ; X and Y together are ( $=O$ ) and  $n=0$

Illustrative of the preparation of the perfluoroalkyl acetals of dialdehydes is that of the  $C_{11}$  trihydrofluoroacetal of tetraethoxypropane. Sixty-four grams of  $C_{11}$  trihydrofluoroalcohol [ $F_2HC(CF_2)_9CH_2OH$ ], about 0.12 mol, were reacted with seven grams of tetraethoxypropane ( $C_2H_5O)_4C_3H_4$ , about 0.032 mol, dissolved in fifty grams of dimethylformamide and 1.0 gram of concentrated sulfuric acid. The mixture was held at 100° C. for two hours, then the ethanol produced and unreacted ethoxypropane were removed under a vacuum. Thereafter at a higher temperature dimethylformamide

was removed by distillation under a vacuum. A residue of 67.3 grams of a waxy solid.



where Q is the perfluoroalkyl radical of the  $C_{11}$  trihydrofluoroalcohol,  $F_2CH(CF_2)_9CH_2-$ , were obtained.

The foregoing reaction is illustrative of the preparation of the perfluoroalkylacetals of dialdehydes by transesterification. However, these perfluoroalkylacetals of dialdehydes can also be made by direct reaction of the perfluoroalkanol and a dialdehyde.

#### EXAMPLE 5

Employing the compounds and concentrations described in Example 2, dispersions are prepared using 0.5% sodium lauryl sulfate as the emulsifier. Concentrated solutions of compounds in dimethylformamide are emulsified in water with the aforementioned emulsifying agent. These emulsions are then applied and dried at room temperature. Excellent soil and water-proofing is obtained. Illustrative of the water-proofing characteristics, the textiles treated with compound 2D has a spray rating of 100 (as hereinafter described). Compounds 2F, 2H, 2J and 2M also give 100 ratings.

#### EXAMPLE 6

Example 1 is repeated except that in place of the fluoroo alcohol used there, 2 mols of trifluoroethanol



are used. Textiles treated with this reaction product exhibit no oil or water-repellency and no soil resistance.

#### EXAMPLE 7

The procedures of Examples 2 and 3 are repeated using the following acetals in the indicated concentrations.

- A. 1% n-hexyl-O O-n-hexyl  
 B. 5% 2-ethyl hexyl-O O-2-ethyl hexyl  
 C. 3% n-hexyl-O O-C2H5  
 D. 1% C2H5O O-C2H5  
 E. 3% C1C2H4O O-C2H4Cl





**11**

- (1) wherein  $Q_1$  is an alkyl group of from 3 to 22, said alkyl having a terminal group selected from the group consisting of  $-\text{CHF}_2$  and  $-\text{CF}_3$  and said alkyl having at least 70 percent of the hydrogen atoms thereof replaced by fluorine atoms,  
 (2)  $Q_2$ ,  $Q_3$  and  $Q_4$  are independently selected from the group consisting of  $Q_1$  fluoroalkyls and alkyl of 6 to 30 carbon atoms,  
 (3) the  $R_1$ 's are independently alkyl of 1 to 4 carbon atoms,  
 (4)  $Z$  is selected from the group consisting of  $OQ_1$  and alkoxy of 1 to 30 carbon atoms, and  
 (5)  $n$  has a value of from 0 to 22.  
 2. Compounds as defined in claim 1 of Formula I.  
 3. Compounds as defined in claim 1 of Formula II.  
 4. Compounds as defined in claim 2 wherein  $Q_2$ ,  $Q_3$  and  $Q_4$  are  $Q_1$  fluoroalkyls.  
 5. Compounds as defined in claim 2 wherein  $Q_2$  is a  $Q_1$  fluoroalkyl and  $Q_3$  and  $Q_4$  are alkyl.  
 6. Compounds as defined in claim 3 wherein  $Z$  is  $OQ_1$ .

5

**12**

7. Compounds as defined in claim 3 wherein  $Z$  is alkoxy of 1 to 4 carbon atoms.  
 8. Compounds as defined in claim 3 wherein  $Z$  is alkoxy of 5 to 30 carbon atoms.

**References Cited****UNITED STATES PATENTS**

|           |         |                            |
|-----------|---------|----------------------------|
| 2,360,957 | 10/1944 | MacDowell et al.           |
| 2,556,312 | 6/1951  | Young.                     |
| 2,802,879 | 8/1957  | Guest et al. ----- 260—602 |
| 2,824,141 | 2/1958  | Zisman.                    |
| 2,988,537 | 6/1961  | Wiley ----- 260—602        |
| 2,883,429 | 4/1959  | Hazeldine.                 |

15 HOWARD T. MARS, Primary Examiner

**U.S. Cl. X.R.**

8—116.4, 120; 106—2, 188, 270, 288; 117—138.8, 139.5, 141, 143, 144; 252—8.6; 260—602